# EUROPEAN PATENT SPECIFICATION

(11) **EP 3 648 117 B1**
(45) Date of publication and mention of the grant of the patent: **14.01.2026**
(21) Application number: 18204086.5
(22) Date of filing: 02.11.2018
(51) Int. Cl.: H01B 7/28, H01B 3/22, H01B 3/30, H01B 3/40, H01B 3/44, H01B 3/46

(54) **ELECTRICAL INSULATION, USE OF AN ELECTRICAL INSULATION, AND METHOD OF PRODUCING AN ELECTRICAL INSULATION**
ELEKTRISCHE ISOLIERUNG, VERWENDUNG EINER ELEKTRISCHEN ISOLIERUNG UND VERFAHREN ZUR HERSTELLUNG EINER ELEKTRISCHEN ISOLIERUNG
ISOLATION ÉLECTRIQUE, UTILISATION D'UNE ISOLATION ÉLECTRIQUE ET PROCÉDÉ DE PRODUCTION D'UNE ISOLATION ÉLECTRIQUE

(43) Date of publication of application: 06.05.2020
(73) Proprietor: Hitachi Energy Ltd, 8050 Zürich (CH)
(72) Inventor: Christen, Thomas, 5413 Birmenstorf (CH); Meier, Patrick, 5603 Staufen (CH); Di-Gianni, Anna, 5405 Dättwil (CH); Krivda, Andrej, 5430 Wettingen (CH)
(74) Representative: Vossius & Partner Patentanwälte Rechtsanwälte mbB

(56) References cited:
- EP-A1- 1 168 372
- WO-A1-2016/170952
- US-A- 3 446 741

## Description

### FIELD OF THE INVENTION

The invention relates to an electrical insulation and methods of using and producing an electrical insulation. The invention relates in particular to an electrical insulation and methods of using and producing an electrical insulation that provide enhanced tolerance to defects.

### BACKGROUND OF THE INVENTION

Electrical insulations are widely used to electrically insulate power system components, such as cables of a transmission line, busbars, transformer components, or other power system components.

An electrical insulation may be based on an electrically insulating material, such as an epoxy resin. An epoxy based electrical insulation can be manufactured by mixing epoxy resin, hardener, accelerator and various fillers. Such an electrical insulation may be susceptible to electrical treeing. Electrical treeing may originate from metallic electrodes or impurities in the insulation, e.g., metallic particles and wires, small pieces of glass, wood or gas bubbles. Electrical treeing is a defect that commonly occurs in the electrical insulation of power system components. Partial discharges may cause a tree-shaped cavity to form in an electrical insulator.

US 6 764 616 B1 discloses a hydrophobic epoxide resin system used as an electrical insulating material.

P. Vijayan and M. A. AlMaadeed, "'Containers' for self-healing epoxy composites and coating: Trends and advances", eXPRESS Polymer Letters Vol.10, No.6 (2016) 506-524 suggests the introduction of a self-healing functionality into an epoxy matrix by using polymer capsules in epoxy composites.

X. J. Ye et al., "Improvement of fatigue resistance of epoxy composite with microencapsulated epoxy-SbF5 self-healing system", eXPRESS Polymer Letters Vol.11, No.11 (2017) 853-862 discloses a technique for rapid retardation and arresting of fatigue cracks that uses, inter alia, microcapsules induced toughening.

EP 1 168 372 A1 discloses a material for self-curing electrical insulations that are capable of restoring hydrophobic characteristics of a surface.

US 3 446 741 A discloses an insulating device and composition.

There is a continued need in the art for an electrical insulation that provides enhanced tolerance to defects, i.e., that is less likely to fail once a defect starts to develop. There is in particular a continued need in the art for an electrical insulation that provides improved robustness to electrical treeing.

Conventional epoxy composite materials are not adequate to provide sufficient resistance to electrical treeing. For illustration, the curing characteristics of the materials described in P. Vijayan and M. A. AlMaadeed, "'Containers' for self-healing epoxy composites and coating: Trends and advances", eXPRESS Polymer Letters Vol.10, No.6 (2016) 506-524 and in X. J. Ye et al., "Improvement of fatigue resistance of epoxy composite with microencapsulated epoxy-SbF5 self-healing system", eXPRESS Polymer Letters Vol.11, No.11 (2017) 853-862 are such that the materials tend to self-cure too rapidly and cannot flow into channels formed by electrical treeing in an electrical insulation. This adversely affects the suitability of the epoxy composite of these documents for mitigating electrical treeing.

### SUMMARY

It is an object of the invention to provide an improved electrical insulation and improved methods that provide enhanced tolerance to at least certain types of defects in the electrical insulation. It is in particular an object to provide an electrical insulation and methods of using and producing the electrical insulation, wherein the electrical insulation provides enhanced robustness against growth of electrical trees in the electrical insulation.

An electrical insulation, its use for impeding growth of an electrical tree, a power system component, and a method of production as recited in the independent claims define the claimed invention. The dependent claims define embodiments of the claimed invention.

The invention provides an electrical insulation in which capsules having a solid shell containing an electrically insulating liquid are provided in an insulating material, such as an epoxy resin, polyurethane resin, polyethylene or other polymeric materials. The insulating material may include optional other fillers. When an electrical tree starts during operation of a power equipment, the electrical tree eventually hits one of the capsules, punctures it, and enables the insulating liquid from the capsule to flow into treeing channels. The electrically insulating liquid flowing into the treeing channels interferes with discharges in the treeing channels and thus significantly slows down the degradation of the electrical insulation.

The capsules may be microcapsules. The microcapsules may have a diameter, measured along the maximum length of the microcapsules, which is not more than 1000 µm, preferably not more than 500 µm, further preferably not more than 100 µm. The microcapsules may have a diameter, measured along the maximum length of the microcapsules, which may be between 2 µm and 1000 µm. The microcapsules may have a diameter, measured along the maximum length of the microcapsules, which may be between 2 µm and 1000 µm, preferably between 2 µm and 500 µm.

An electrical insulation according to an embodiment comprises an electrically insulating material and an electrical tree inhibiting material in the electrically insulating material. The electrical tree inhibiting material comprises a plurality of capsules having a shell and an electrically insulating liquid within the shell. The shell is formed of a multi-layer system having several layers, and the several layers comprise a gelatin and/or resorcinol coating.

The electrically insulating material may be a solid.

The shell of the capsules may be a solid different from the electrically insulating material. The shell of the capsules may be configured to rupture in response to the mechanical stress and/or electrical field induced by electrical treeing.

The electrically insulating liquid may be or may comprise oil or a blend of oils. The electrically insulating liquid may be or may comprise a silicone oil, a blend of silicone oils, a mineral transformer oil, a blend of mineral transformer oils and/or a vegetable oil, or a blend of vegetable oils. The electrically insulating liquid may comprise a blend of the mentioned oils.

The electrically insulating liquid may have a resistivity from 10³ Ω m to 10²⁰ Ω m.

The electrically insulating liquid may have a resistivity from 10³ Ω m to 10²⁰ Ω m at 25°C.

The electrically insulating liquid may have dielectric permittivity from 1 to 50 at 25°C and at 50 Hz.

The electrically insulating liquid may have a low viscosity.

The electrically insulating liquid may have a dynamic viscosity of less than 100000 mm²/s at 25°C (measured according to DIN 53019).

The electrically insulating liquid may have a dynamic viscosity of more than 0.01 mm²/s at 25°C (measured according to DIN 53019).

The electrically insulating liquid may have a dynamic viscosity of 0.01 mm²/s to 100000 mm²/s, preferably of 1 mm²/s to 10000 mm²/s at 25°C (measured according to DIN 53019).

The electrically insulating liquid may be a non-UV-curing electrically insulating liquid.

The electrically insulating liquid may be a non-self-curing electrically insulating liquid.

The electrically insulating liquid may contain fillers. The fillers within the insulating liquid contained in the capsules may be nanoparticles.

The capsules may be microcapsules.

A root-mean-square value of a maximum diameter of the capsules may be not more than 1000 µm, preferably not more than 500 µm, preferably not more than 100 µm.

A root-mean-square value of a maximum diameter of the capsules may be between 2 µm and 1000 µm, optionally between 2 µm and 500 µm.

The shell may comprise melamine formaldehyde or polyoxymethylene urea or other materials. The shell may contain fillers.

The shell may have a wall thickness in the range from 0.1 µm to 100 µm.

The shell may be free of fillers such as TiO₂.

The shell may be free of TiO₂.

The capsules may be dispersed in the electrically insulating material.

The electrical insulation may comprise at least 1 wt-% of the capsules and/or at least 2 vol-% of the capsules.

The electrical insulation may comprise between 1 wt-% and 30 wt-% of the capsules.

The electrical insulation may comprise between 2 vol-% and 50 vol-% of the capsules.

The electrically insulating material may be or may comprise an epoxy resin, polyurethane resin, polyethylene or other polymeric materials.

The electrically insulating material may have fillers other than the capsules. The fillers may comprise an anti-settling agent (a sag resistance agent). The anti-settling agent or sag resistance agent may be operative to prevent or reduce settling of the capsules under influence of gravity in a mixture that includes the electrically insulating material in liquid phase, the capsules, and the anti-settling agent or sag resistance agent.

A power system component according to an embodiment comprises an electrical component, in particular a conductor, and the electrical insulation according to an embodiment.

The power system component may be a power transmission cable, in particular an underground cable.

The power system component may be a busbar.

The power system component may be a transformer.

The power system component may be a circuit breaker.

The power system component may be a switchgear.

The power system component may be an insulating spacer.

The power system component may be a switch.

The power system component may be a motor.

The power system component may be a generator.

The power system component may be a bushing.

Also disclosed is a power system that comprises a power system component having the electrical insulation according to an embodiment. The power system may be a medium or high voltage power transmission system.

In a use of the electrical insulation according to an embodiment for impeding growth of an electrical tree, the shell of at least one capsule ruptures to release the electrically insulating liquid into a cavity formed by an electrical tree when the electrical tree impinges onto the shell of the at least one capsule. The electrically insulating liquid flows into the cavity of the electrical tree and impedes growth of the electrical tree. The electrical insulation may be the electrical insulation according to any claimed embodiment disclosed herein.

A method of producing an electrical insulation according to an embodiment comprises forming a mixture comprising a polymeric material and a plurality of capsules in the polymeric material, wherein each of the capsules has a shell and an electrically insulating liquid within the shell, the shell being formed of a multi-layer system having several layers, wherein the several layers comprise a gelatin and/or resorcinol coating. The claimed method further comprises processing the mixture into a solid electrical insulation.

The polymeric material may comprise or may be a thermoset or thermoplast or elastomer or mixture or blend or co-polymer of these polymers.

The polymeric material may be or may comprise an epoxy resin, polyurethane resin, polyethylene or other polymeric materials.

Processing the mixture into a solid electrical insulation may comprise effecting a cross-linking reaction, curing, melting and/or otherwise processing the polymeric material.

The mixture may optionally comprise fillers other than the plurality of capsules.

The fillers may comprise an anti-settling agent (a sag resistance agent). The anti-settling agent or sag resistance agent may be operative to prevent or reduce settling of the capsules under influence of gravity in the mixture that includes the electrically insulating material in liquid phase, the capsules, and the anti-settling agent or sag resistance agent.

The shell of the capsules in the mixture may be a solid. The shell of the capsules may be configured to rupture in response to the mechanical stress and/or electrical field induced by electrical treeing.

The electrically insulating liquid contained within the capsules in the mixture may be or may comprise a silicone oil, a blend of silicone oils, a mineral transformer oil, a blend of mineral transformer oils and/or a vegetable oil or a blend of vegetable oils, or a blend of these oils.

The electrically insulating liquid contained within the capsules in the mixture may have a resistivity from 10³ Ω m to 10²⁰ Ω m.

The electrically insulating liquid contained within the capsules in the mixture may have a resistivity from 10³ Ω m to 10²⁰ Ω m at 25°C.

The electrically insulating liquid contained within the capsules in the mixture may have dielectric permittivity from 1 to 50 at 25°C and at 50 Hz.

The electrically insulating liquid contained within the capsules in the mixture may have a low viscosity.

The electrically insulating liquid contained within the capsules in the mixture may have a dynamic viscosity of less than 100000 mm²/s at 25°C (measured according to DIN 53019).

The electrically insulating liquid contained within the capsules in the mixture may have a dynamic viscosity of more than 0.01 mm²/s at 25°C (measured according to DIN 53019).

The electrically insulating liquid may have a dynamic viscosity of 0.01 mm²/s to 100000 mm²/s, preferably of 1 mm²/s to 10000 mm²/s at 25°C (measured according to DIN 53019).

The electrically insulating liquid contained within the capsules in the mixture may be a non-UV-curing electrically insulating liquid.

The electrically insulating liquid contained within the capsules in the mixture may be a non-self-curing electrically insulating liquid.

The electrically insulating liquid contained within the capsules in the mixture may contain fillers. The fillers within the insulating liquid contained in the capsules may be nanoparticles.

The capsules in the mixture may be microcapsules.

A root-mean-square value of a maximum diameter of the capsules may be not more than 1000 µm, preferably not more than 500 µm, preferably not more than 100 µm.

A root-mean-square value of a maximum diameter of the capsules may be between 2 µm and 1000 µm, optionally between 2 µm and 500 µm.

The shell of the capsules in the mixture may comprise melamine formaldehyde or polyoxymethylene urea or other materials.

The shell of the capsules in the mixture may contain fillers.

The shell of the capsules in the mixture may be free of fillers such as TiO₂.

The shell of the capsules in the mixture may have a wall thickness in the range from 0.1 µm to 100 µm.

The mixture may comprise at least 1 wt-% of the capsules and/or at least 2 vol-% of the capsules. The method may comprise causing a cross-linking reaction of the polymeric material.

The mixture may comprise a hardener and/or an accelerator to facilitate the cross-linking reaction.

The method may further comprise disposing the cured mixture, optionally after further post-processing, adjacent an electrical component, in particular adjacent a conductor, of a power system component.

The cured mixture may comprise between 1 wt-% and 30 wt-% of the capsules.

The cured mixture may comprise between 2 vol-% and 50 vol-% of the capsules.

The power system component may be a power transmission cable, a busbar, a transformer, a circuit breaker, a switchgear, a switch, a spacer, a bushing, a motor, or a generator.

Various effects are attained by the electrical insulation and methods according to embodiments. For illustration, when an electrical tree hits a capsule, rupture of the shell causes the electrically insulating liquid from the capsule to flow into one or several treeing channels and interfere with the discharges in the treeing channels. A low viscosity of the electrically insulating liquid in the capsules, e.g., the low viscosity of a silicone oil, blend of silicone oils, mineral transformer oil(s) and/or vegetable oil(s) may assist the capability of the electrically insulating liquid to flow into the treeing channels. Use of a non-self-curing and non-UV-curing the electrically insulating liquid in the capsules ensures that the electrically insulating liquid in the capsules remains capable of flowing into the treeing channels.

The electrical insulation according to embodiments provides enhanced tolerance to defects in the sense that, even when electrical treeing starts, the time to breakdown of the electrical insulation is extended compared to conventional electrical insulations that are based on similar electrically insulating materials, such as epoxy resins.

The electrical insulator may be used for power system components of high or medium voltage power systems, without being limited thereto.

The electrical insulator may be used for a power generation or power transmission system, without being limited thereto.

### BRIEF DESCRIPTION OF THE DRAWINGS

The subject-matter of the invention will be explained in more detail with reference to preferred exemplary embodiments which are illustrated in the attached drawings, in which:
Figure 1 is a schematic representation of a power system component comprising an electric insulation according to an embodiment.
Figure 2 is a cross-sectional view of a capsule of an electrical insulator according to an embodiment.
Figure 3 is a cross-sectional view of a capsule of an electrical insulator according to an embodiment.
Figure 4 is a cross-sectional view of a capsule of an electrical insulator according to an embodiment.
Figure 5 is a cross-sectional view of a capsule of an electrical insulator according to an embodiment.
Figures 6 and 7 are cross-sectional views of an electrical insulator according to an embodiment.
Figure 8 is a cross-sectional view of a test specimen.

### DETAILED DESCRIPTION OF EMBODIMENTS

Exemplary embodiments of the invention will be described with reference to the drawings in which identical or similar reference signs designate identical or similar elements. Some embodiments will be described in the context of specific exemplary electrically insulating materials that may be based on an epoxy resin, polyurethane, polyethylene or other polymeric materials, with reference to exemplary fillers, and with reference to specific exemplary capsules.

While some embodiments will be described in the context of specific exemplary power system components, such as cables of a transmission line, busbars, or conductors in transformers, the electrical insulator according to embodiments may be used in a wide variety of other applications. The features of embodiments may be combined with each other, unless specifically noted otherwise.

Fig. 1 is a schematic representation of a power system component 10 comprising an electrical insulator according to an embodiment. The power system component 10 may be a component of a power generation or power transmission system. The power system component 10 may be a component of a high or medium voltage power system. The power system component 10 may be a power transmission cable, a busbar, a transformer, a circuit breaker, a switchgear, a switch, a motor, a generator. Exemplary power system components 10 include primary or secondary gas insulated switchgear, live tank breakers, dead tank breakers, generator circuit breakers, instrument transformers, other transformers, coils, bushings, sensors, railway power components, vacuum poles, or vacuum interrupters, without being limited thereto.

The power system component 10 comprises an electrical component 11, which may in particular be a conductor, and an electrical insulation 20. The electrical insulation 20 may be disposed to cover at least part of the electrical component 11.

The electrical insulation 20 according to embodiments is a composite system. The electrical insulation 20 may comprise
- an electrically insulating material 21, which may comprise or which may be an epoxy resin, polyurethane, polyethylene and/or other polymer,
- capsules 30 that are dispersed in the electrically insulating material 21, and which will be described in more detail below,
- optional fillers such as sag resistance or anti-settling agents that may be used in the production process to ensure a uniform distribution of the capsules 30, and
- optional hardeners and/or accelerators.

As compared to conventional electrical insulations, the electrical insulation 20 comprises capsules 30 that are dispersed in a solid electrically insulating material 21. The capsules 30 are operative to inhibit growth of an electrical tree, thereby enhancing the defect tolerance of the electrical insulation 20.

The capsules 30 may respectively be microcapsules. The capsules 30 may respectively have a mean diameter of less than 1000 µm, preferably less than 500 µm, preferably less than 100 µm. The capsules 30 may respectively have a mean diameter from 2 µm to 1000 µm, optionally from 2 µm to 500 µm.

The capsules 30 may be evenly distributed throughout the electrically insulating material 21. The capsules 30 may be distributed throughout the electrically insulating material 21 such that any volume of 1 cm³ of the electrical insulator includes from 2 vol-% to 50 vol-% of the capsules.

The electrical insulation may comprise at least 1 wt-% of the capsules and/or at least 2 vol-% of the capsules. The electrical insulation may comprise 7 wt-% or more of the capsules. Alternatively or additionally, the electrical insulation may comprise 2 vol-% or more of the capsules. This ensures that a release of electrically insulating liquid from the capsule into a cavity formed by an electrical tree will mitigate further growth of the electrical tree at an early stage, thereby increasing robustness of the electrical insulation against electrical treeing.

Figures 2 to 5 illustrate exemplary capsules 30. The capsules 30 may respectively be configured as microcapsules. The capsules 30 may respectively have a solid shell 31 that defines an interior volume 32. The capsules 30 respectively have a silicone oil 36 or other electrically insulating, low-viscosity liquid in the interior volume 32 defined by the shell 31. For illustration, a silicone oil, mineral transformer oil, vegetable oil or a blend of several such oils that is electrically insulating may be provided in the interior volume 32.

By using an electrical insulation 20 that comprises capsules 30 having a shell 31 made of, for example, melamine formaldehyde or polyoxymethylene urea or other suitable shell material, and filled with an electrically insulating liquid or a blend of several insulating liquids 36 in the electrically insulating material 21, the growth of electrical trees in the electrical insulation 20 can be stopped or impeded. The electrically insulating liquid or a blend of several insulating liquids may include low viscosity silicone oil(s), mineral transformer oil(s), vegetable oil(s) or a blend of such oils.

The electrically insulating liquid may have a resistivity from 10³ Ω m to 10²⁰ Ω m at 25°C. The electrically insulating liquid may have dielectric permittivity from 1 to 50 at 25°C and at 50 Hz.

During use of the electrical insulation 20, partial discharges may cause electrical treeing to start. When the electrical tree impinges on one or several of the capsules 30, it causes the shell of the capsule(s) 30 to rupture, releasing the electrically insulating liquid 36 into one or several channels of the electrical tree.

The electrically insulating liquid 36 may be or may comprise a silicone oil, mineral transformer oil, vegetable oil or a blend of such oils. The electrically insulating liquid 36 may have a dynamic viscosity of equal to or less than 100000 mm²/s at 25°C (measured according to DIN 53019) and of equal to or more than 0.01 mm²/s at 25°C (measured according to DIN 53019). The electrically insulating liquid 36 may be or may comprise a blend of various silicone liquids, or other oils, mixed so as to attain a dynamic viscosity of equal to or less than 100000 mm²/s and equal to or more than 0.01 mm²/s (measured according to DIN 53019). The electrically insulating liquid 36 may preferably have a dynamic viscosity at 25°C (measured according to DIN 53019) which is from 1 mm²/s to 10000 mm²/s.

The electrically insulating liquid 36 may be or may comprise dimethyl polysiloxanes, mineral transformer oils, vegetable oils, or blends of several such oils.

The shell 31 may be made of a material which is responsive to mechanical stress in the electrically insulating material 21, causing the shell 31 to rupture in response to the electromechanical stress caused by the branches of an electrical tree. Alternatively or additionally, the shell 31 may be made of a material which is responsive to the electric field caused by partial discharges in electrical treeing, causing the shell 31 to rupture in response to the electrical field caused by electrical treeing.

According to the claimed invention, multilayer shell constructions are used, as explained with reference to Figures 3 and 4.

Figure 3 illustrates an exemplary capsule 30. The capsule 30 has a solid shell formed of an inner layer 33 and an outer coating 34. The inner layer 33 may be made of, for example, melamine formaldehyde or polyoxymethylene urea or other suitable shell material. The outer coating 34 is made of or comprises a gelatin coating and/or a resorcinol coating.

Figure 4 illustrates an exemplary capsule 30. The capsule 30 has a solid shell formed of an inner layer 33 and plural coating layers 34, 35. The inner layer 33 may be made of, for example, melamine formaldehyde or polyoxymethylene urea or other suitable shell material. The coating layer 34 is made of or comprises a gelatin coating or another material. The coating layer 35 is made of or comprises a resorcinol coating or another material.

In the capsules 30 explained with reference to Figures 2 to 4, the shell 31 or each layer 33, 34, 35 of the shell may completely surround the interior volume 32, so as to retain the electrically insulating liquid therein.

The capsules 30 may respectively have a mean maximum diameter of equal to or less than 1000 µm, preferably of equal to or less than 500 µm. The capsules 30 may respectively have a mean maximum diameter of equal to or more than 2 µm. The determination of the mean maximum diameter will be exemplarily explained with reference to Figure 5. A line 38 is determined such that a distance 39 between the intersection of the line 38 and the outermost surface of the shell is maximum. The distance 39 is referred to as maximum diameter. The maximum diameters determined for at least ten capsules is averaged to determine the mean maximum diameter.

Figures 6 and 7 are cross-sectional views of an electrical insulation 20 according to an embodiment, which illustrate the operation of the electrical insulation 20. Figure 6 depicts the electrical insulation in a state in which branches 41a, 41b of a cavity 40 formed by an electrical tree impinge on capsules 30a, 30b embedded within the electrically insulating material 21. When the branches 41a, 41b formed by the electrical tree impinge on the capsules 30a, 30b, the shell of the capsules is ruptured. This releases the electrically insulating liquid from the capsules 30a, 30b into the branches 41a, 41b of the cavity 40. The electrically insulating liquid impedes growth of the electrical tree. For illustration, the electrically insulating liquid may mitigate the risk of further partial discharges occurring.

In order to manufacture the electrical insulation according to an embodiment, a polymeric material in the liquid phase, such as a liquid epoxy resin, polyethylene, polyurethane or other polymeric material, may be mixed with capsules 30 having a shell and an electrically insulating liquid within the shell. Polymeric materials other than epoxy resin may be used. For illustration, the polymeric material may comprise or may be a thermoset or thermoplast or elastomer or mixture or blend or co-polymer of these polymers.

The mixture may comprise optional additional fillers, optional hardeners, and/or optional accelerators.

The mixture may comprise at least 1 wt-% of the capsules and/or at least 2 vol-% of the capsules. The capsules may have the configuration explained with reference to Figures 1 to 7 above.

The mixture may comprise a sag resistance or anti-settling agent that mitigates the risk of the capsules settling in the mixture. The mixture may comprise 0.05 to 10 wt-% of anti-settling agent. The epoxy resin may be processed into a solid to form the electrical insulation. For illustration, curing or other hardening techniques may be employed.

The method may comprise optional post-processing after hardening the mixture. The method may comprise applying the electrical insulation to an electrical component, in particular a conductor, of a power system component.

The electrical insulation according to embodiments provides enhanced defect tolerance compared to conventional electrical insulations, in particular as regards the time to breakdown by electrical treeing.

Tests were performed that evidence the improved characteristics of the electrical insulation according to embodiments.

Figure 8 shows a test specimen having a body of an electrical insulation 50. A planar electrode 51 is applied on one face of the body 50. A pin electrode 52 is inserted on the opposite face. Polydimethylsiloxan (PDMS) 53 may be applied to the face on which the pin electrode 52 enters the body 50.

Comparative samples A and inventive samples B were produced to have the following composition of the body 50:
Comparative sample A: up to 65% standard silica SiO₂ and epoxy resin.

Inventive sample B: up to 65 wt-% standard silica SiO₂; between 0.01 to 10 wt-% of anti-settling agent and 1-20 wt-% of microcapsules; and epoxy resin. The total weight of fillers in inventive samples of type B always matched the weight of fillers in comparative samples of type A.

Twelve test specimens were respectively produced for sample A and twenty four for sample B.

The time to breakdown was measured. The same voltage was applied to the test specimens of comparative sample A and the test specimens of inventive sample B.

The measured time to breakdown for the comparative samples A is summarized in the following Table 1:

**Table 1**

| Sample type | time to breakdown [hours] |
|---|---|
| A | 90 |
| A | 388 |
| A | 455 |
| A | 482 |
| A | 502 |
| A | 559 |
| A | 617 |
| A | 764 |
| A | 867 |
| A | 980 |
| A | 1273 |
| A | 1287 |

None of twenty four inventive samples B failed while being under voltage for more than 1900 hours. Twelve inventive samples B were operating for more than 3400 hours without failure at the time of drafting of this application.

The electrical insulation according to embodiments which comprises capsules filled with an electrically insulating liquid as an electrical tree inhibiting material provides various effects and advantages. Robustness to defects such as electrical trees is enhanced. Capsules filled with low-viscosity insulating liquids, e.g., silicone oils, mineral transformer oils, and/or vegetable oils or blends thereof have various desirable characteristics. The silicone oil has a lower carbon content than, e.g., the epoxy. A range of viscosities is available, facilitating the selection of a low-viscosity liquid that can easily and rapidly flow into the branches of an electrical tree. Silicone oil turns into silica sand during decomposition.

The electrically insulating liquid contained within the capsules may contain fillers, such as nanoparticles.

When the electrically insulating liquid in the capsules is non-UV-curing, various further desirable effects are attained. UV curing systems are prone to curing by themselves without action of UV light from partial discharges in the treeing channels within several weeks. The non-UV-curing electrically insulating liquids used in embodiments of the electrical insulation are suitable for use on power system components with an expected lifetime of 10 to 40 years.

An electrical insulation and methods according to the invention may be used in association with a power system component, e.g., a power generation or power transmission system. The electrical insulation may in particular be used for isolating a power transmission cable, a busbar, a transformer, a circuit breaker, a switchgear, a switch, a bushing, a spacer, a motor, or a generator, without being limited thereto. Exemplary power system components that may comprise the electrical insulation according to an embodiment may include primary or secondary gas insulated switchgear, live tank breakers, dead tank breakers, generator circuit breakers, instrument transformers, other transformers, coils, bushings, sensors, railway power components, vacuum poles, or vacuum interrupters.

## Claims

1. An electrical insulation (20), comprising:
an electrically insulating material (21), and
an electrical tree inhibiting material in the electrically insulating material (21), the electrical tree inhibiting material comprising a plurality of capsules (30) having a shell (31; 33, 34; 33-35) and an electrically insulating liquid (36) within the shell (31; 33, 34; 33-35),
**characterized in that**
the shell (33, 34; 33-35) is formed of a multi-layer system having several layers,
wherein the several layers comprise a gelatin and/or resorcinol coating.

2. The electrical insulation (20) of claim 1, wherein the electrically insulating liquid (36) comprises a silicone oil, a mineral transformer oil or a vegetable oil, or their blends, optionally wherein the electrically insulating liquid contains one or several fillers, optionally wherein the one or several fillers comprises a sag resistance agent which is operative to prevent or reduce settling of the capsules under influence of gravity in a mixture that includes the electrically insulating material in liquid phase, the capsules, and the sag resistance agent.

3. The electrical insulation (20) of claim 1 or claim 2, wherein the electrically insulating liquid (36) has a viscosity at 25°C measured according to DIN 53019 of equal to or less than 100000 mm²/s, preferably of equal to or less than 10000 mm²/s.

4. The electrical insulation (20) of any one of the preceding claims, wherein the electrically insulating liquid (36) has a viscosity at 25°C measured according to DIN 53019 of more than 0.01 mm²/s, preferably of more than 1 mm²/s.

5. The electrical insulation (20) of any one of the preceding claims, wherein the electrically insulating liquid (36) is a non-UV-curing electrically insulating liquid (36).

6. The electrical insulation (20) of any one of the preceding claims, wherein a root-mean-square value of a maximum diameter (39) of the capsules (30) is not more than 1000 µm, preferably not more than 500 µm, further preferably not more than 100 µm.

7. The electrical insulation (20) of any one of the preceding claims, wherein the shell (31; 33, 34; 33-35) comprises melamine formaldehyde or polyoxymethylene urea or other materials.

8. The electrical insulation (20) of any one of the preceding claims, wherein the shell (31; 33, 34; 33-35) is free of TiO₂ and/or wherein the shell (31) contains one or several fillers.

9. The electrical insulation (20) of any one of the preceding claims, wherein the capsules (30) are dispersed in the electrically insulating material (21).

10. The electrical insulation (20) of any one of the preceding claims, wherein the electrical insulation (20) comprises at least 1 wt-% of the capsules (30) and/or at least 2 vol-% of the capsules (30).

11. The electrical insulation (20) of any one of the preceding claims, wherein the electrically insulating material (21) is an epoxy resin or comprises an epoxy resin, polyurethane or polyethylene or other polymer(s).

12. A power system component (10), comprising:
an electrical component (11), in particular a conductor, and
the electrical insulation (20) according to any one of the preceding claims.

13. The power system component (10) according to claim 12, wherein the power system component (10) is a power transmission cable, a busbar, a transformer, a circuit breaker, a switchgear, a switch, a bushing, a spacer, a motor, or a generator.

14. Use of the electrical insulation (20) of any one of claims 1 to 11 for impeding growth of an electrical tree, wherein the shell (31; 33, 34; 33-35) of at least one capsule (30) ruptures to release the electrically insulating liquid (36) into a cavity (40) formed by an electrical tree when the electrical tree impinges onto the shell (31; 33, 34; 33-35) of the at least one capsule, such that the electrically insulating liquid (36) flows into the cavity (40) formed by the electrical tree and thereby impedes growth of the electrical tree (40).

15. A method of producing an electrical insulation (20), the method comprising:
forming a mixture comprising a polymeric material and a plurality of capsules (30) in the polymeric material, wherein each of the capsules (30) has a shell (31; 33, 34; 33-35) and an electrically insulating liquid (36) within the shell (31; 33, 34; 33-35), and
processing the mixture into a solid electrical insulation (20),
**characterized in that**
the shell (33, 34; 33-35) is formed of a multi-layer system having several layers,
wherein the several layers comprise a gelatin and/or resorcinol coating.

## Patentansprüche

1. Elektrische Isolierung (20), umfassend:
ein elektrisch isolierendes Material (21), und
ein Material zur Hemmung eines elektrischen Baums in dem elektrisch isolierenden Material (21), wobei das Material zur Hemmung des elektrischen Baums eine Mehrzahl von Kapseln (30) aufweist, die eine Hülle (31; 33, 34; 33-35) und eine elektrisch isolierende Flüssigkeit (36) innerhalb der Hülle (31; 33, 34; 33-35) aufweisen,
**dadurch gekennzeichnet, dass**
die Hülle (33, 34; 33-35) aus einem Mehrschichtsystem gebildet ist, das mehrere Schichten hat,
wobei die mehreren Schichten eine Gelatine- und/oder Resorcinbeschichtung umfassen.

2. Elektrische Isolierung (20) nach Anspruch 1, wobei die elektrisch isolierende Flüssigkeit (36) ein Silikonöl, ein mineralisches Transformatoröl oder ein Pflanzenöl oder deren Mischungen umfasst, wobei optional die elektrisch isolierende Flüssigkeit einen oder mehrere Füllstoffe enthält, wobei optional der eine oder die mehreren Füllstoffe ein Absackverhütungsmittel umfassen, das wirksam ist, ein Absetzen der Kapseln unter dem Einfluss der Schwerkraft in einer Mischung, die das elektrisch isolierende Material in flüssiger Phase, die Kapseln und das Absackverhütungsmittel umfasst, zu verhindern oder zu reduzieren.

3. Elektrische Isolierung (20) nach Anspruch 1 oder Anspruch 2, wobei die elektrisch isolierende Flüssigkeit (36) bei 25 °C eine Viskosität von gleich oder weniger als 100 000 mm²/s, vorzugsweise von gleich oder weniger als 10000 mm²/s, gemessen nach DIN 53019, aufweist.

4. Elektrische Isolierung (20) nach irgendeinem der vorhergehenden Ansprüche, wobei die elektrisch isolierende Flüssigkeit (36) bei 25 °C eine Viskosität von mehr als 0,01 mm²/s, vorzugsweise von mehr als 1 mm²/s, gemessen nach DIN 53019, aufweist.

5. Elektrische Isolierung (20) nach irgendeinem der vorhergehenden Ansprüche, wobei die elektrisch isolierende Flüssigkeit (36) eine nicht-UV-härtende elektrisch isolierende Flüssigkeit (36) ist.

6. Elektrische Isolierung (20) nach irgendeinem der vorhergehenden Ansprüche, wobei ein Wert des quadratischen Mittels eines maximalen Durchmessers (39) der Kapseln (30) nicht mehr als 1000 µm, vorzugsweise nicht mehr als 500 µm, noch bevorzugter nicht mehr als 100 µm, beträgt.

7. Elektrische Isolierung (20) nach irgendeinem der vorhergehenden Ansprüche, wobei die Hülle (31; 33, 34; 33-35) Melaminformaldehyd oder Polyoxymethylenharnstoff oder andere Materialien umfasst.

8. Elektrische Isolierung (20) nach irgendeinem der vorhergehenden Ansprüche, wobei die Hülle (31; 33, 34; 33-35) frei von TiO₂ ist und/oder wobei die Hülle (31) einen oder mehrere Füllstoffe enthält.

9. Elektrische Isolierung (20) nach irgendeinem der vorhergehenden Ansprüche, wobei die Kapseln (30) in dem elektrisch isolierenden Material (21) dispergiert sind.

10. Elektrische Isolierung (20) nach irgendeinem der vorhergehenden Ansprüche, wobei die elektrische Isolierung (20) mindestens 1 Gew.-% an den Kapseln (30) und/oder mindestens 2 Vol.-% an den Kapseln (30) umfasst.

11. Elektrische Isolierung (20) nach irgendeinem der vorhergehenden Ansprüche, wobei das elektrisch isolierende Material (21) ein Epoxidharz ist oder ein Epoxidharz, Polyurethan oder Polyethylen oder ein oder mehrere andere Polymere umfasst.

12. Leistungssystemkomponente (10), umfassend:
eine elektrische Komponente (11), insbesondere einen Leiter, und
die elektrische Isolierung (20) nach irgendeinem der vorhergehenden Ansprüche.

13. Leistungssystemkomponente (10) nach Anspruch 12, wobei die Leistungssystemkomponente (10) ein Leistungsübertragungskabel, eine Sammelschiene, ein Transformator, ein Leistungsschalter, eine Schaltanlage, ein Schalter, eine Durchführung, ein Abstandshalter, ein Motor, oder ein Generator ist.

14. Verwendung der elektrischen Isolierung (20) nach irgendeinem der Ansprüche 1 bis 11 zum Behindern eines Wachstums eines elektrischen Baums, wobei die Hülle (31; 33, 34; 33-35) zumindest einer Kapsel (30) reißt, um die elektrisch isolierende Flüssigkeit (36) in einen Hohlraum (40) freizusetzen, der durch einen elektrischen Baum gebildet wird, wenn der elektrische Baum auf die Hülle (31; 33, 34; 33-35) der mindestens einen Kapsel trifft, so dass die elektrisch isolierende Flüssigkeit (36) in den Hohlraum (40) fließt, der durch den elektrischen Baum gebildet wird, und dadurch das Wachstum des elektrischen Baums (40) behindert.

15. Verfahren zur Herstellung einer elektrischen Isolierung (20), wobei das Verfahren umfasst:
Bilden einer Mischung, die ein Polymermaterial und eine Mehrzahl von Kapseln (30) in dem Polymermaterial umfasst, wobei jede der Kapseln (30) eine Hülle (31; 33, 34; 33-35) und eine elektrisch isolierende Flüssigkeit (36) innerhalb der Hülle (31; 33, 34; 33-35) aufweist, und
Verarbeiten der Mischung zu einer festen elektrischen Isolierung (20),
**dadurch gekennzeichnet, dass**
die Hülle (33, 34; 33-35) aus einem Mehrschichtsystem gebildet ist, das mehrere Schichten hat,
wobei die mehreren Schichten eine Gelatine- und/oder Resorcinbeschichtung umfassen.

## Revendications

1. Isolation électrique (20), comprenant :
un matériau électriquement isolant (21), et
un matériau inhibant les arborescences électriques dans le matériau électriquement isolant (21), le matériau inhibant les arborescences électriques comprenant une pluralité de capsules (30) ayant une coque (31 ; 33, 34 ; 33-35) et un liquide électriquement isolant (36) à l'intérieur de la coque (31 ; 33, 34 ; 33-35), **caractérisée en ce que**
la coque (33, 34 ; 33-35) est constituée d'un système multicouche comportant plusieurs couches,
les couches comprenant un revêtement de gélatine et/ou de résorcinol.

2. Isolation électrique (20) de la revendication 1, dans laquelle le liquide électriquement isolant (36) comprend une huile de silicone, une huile minérale de transformateur ou une huile végétale, ou un mélange de celles-ci, éventuellement dans laquelle le liquide électriquement isolant contient une ou plusieurs charges, éventuellement dans laquelle la ou les charges comprennent un agent de résistance à l'affaissement qui sert à empêcher ou réduire la sédimentation des capsules sous l'influence de la gravité dans un mélange qui comporte le matériau électriquement isolant en phase liquide, les capsules, et l'agent de résistance à l'affaissement.

3. Isolation électrique (20) de la revendication 1 ou la revendication 2, dans laquelle le liquide électriquement isolant (36) présente une viscosité à 25 °C mesurée conformément à la norme DIN 53019 égale ou inférieure à 100 000 mm²/s, de préférence égale ou inférieure à 10 000 mm²/s.

4. Isolation électrique (20) de l'une quelconque des revendications précédentes, dans laquelle le liquide électriquement isolant (36) présente une viscosité à 25 °C mesurée conformément à la norme DIN 53019 supérieure à 0,01 mm²/s, de préférence supérieure à 1 mm²/s.

5. Isolation électrique (20) de l'une quelconque des revendications précédentes, dans laquelle le liquide électriquement isolant (36) est un liquide électriquement isolant (36) ne durcissant pas aux UV.

6. Isolation électrique (20) de l'une quelconque des revendications précédentes, dans laquelle une valeur moyenne quadratique d'un diamètre maximal (39) des capsules (30) ne dépasse pas 1000 µm, de préférence ne dépasse pas 500 µm, mieux encore ne dépasse pas 100 µm.

7. Isolation électrique (20) de l'une quelconque des revendications précédentes, dans laquelle la coque (31 ; 33, 34 ; 33-35) comprend de la résine mélamine-formaldéhyde ou de la polyoxyméthylène-urée, ou d'autres matériaux.

8. Isolation électrique (20) de l'une quelconque des revendications précédentes, dans laquelle la coque (31 ; 33, 34 ; 33-35) est dépourvue de TiO₂ et/ou dans laquelle la coque (31) contient une ou plusieurs charges.

9. Isolation électrique (20) de l'une quelconque des revendications précédentes, dans laquelle les capsules (30) sont dispersées dans le matériau électriquement isolant (21).

10. Isolation électrique (20) de l'une quelconque des revendications précédentes, l'isolation électrique (20) comprenant au moins 1 % en poids des capsules (30) et/ou au moins 2 % en volume des capsules (30).

11. Isolation électrique (20) de l'une quelconque des revendications précédentes, dans laquelle le matériau électriquement isolant (21) est une résine époxy ou comprend une résine époxy, un polyuréthane ou un polyéthylène, ou un ou plusieurs autres polymères.

12. Composant de système de puissance (10), comprenant :
un composant électrique (11), en particulier un conducteur, et
l'isolation électrique (20) selon l'une quelconque des revendications précédentes,

13. Composant de système de puissance (10) selon la revendication 12, le composant de système de puissance (10) étant un câble de transmission de puissance, une barre de distribution, un transformateur, un disjoncteur, un appareillage de commutation, un commutateur, une traversée, une entretoise, un moteur, ou un générateur.

14. Utilisation de l'isolation électrique (20) de l'une quelconque des revendications 1 à 11 pour empêcher la croissance d'une arborescence électrique, dans laquelle la coque (31 ; 33, 34 ; 33-35) d'au moins une capsule (30) se rompt pour libérer le liquide électriquement isolant (36) dans une cavité (40) formée par une arborescence électrique lorsque l'arborescence électrique heurte la coque (31 ; 33, 34; 33-35) de l'au moins une capsule, de sorte que le liquide électriquement isolant (36) s'écoule dans la cavité (40) formée par l'arborescence électrique et empêche ainsi la croissance de l'arborescence électrique (40).

15. Procédé de production d'une isolation électrique (20), le procédé comprenant :
la formation d'un mélange comprenant un matériau polymère et une pluralité de capsules (30) dans le matériau polymère, chacune des capsules (30) comportant une coque (31 ; 33, 34 ; 33-35) et un liquide électriquement isolant (36) à l'intérieur de la coque (31 ; 33, 34 ; 33-35), et
la transformation du mélange en une isolation électrique solide (20),
**caractérisé en ce que**
la coque (33, 34 ; 33-35) est constituée d'un système multicouche comportant plusieurs couches,
les couches comprenant un revêtement de gélatine et/ou de résorcinol.
